

# UNITED STATES PATENT OFFICE.

MATAICHI YASUDA, OF KOISHIGAWA, TOKYO, JAPAN.

## COMPOSITION FOR POLISHING IRON.

1,216,643.

Specification of Letters Patent. Patented Feb. 20, 1917.

No Drawing.

Application filed March 14, 1914. Serial No. 824,782.

To all whom it may concern:

Be it known that I, MATAICHI YASUDA, a subject of the Emperor of Japan, residing at Koishigawa, Tokyo, in the Empire of Japan, 5 have invented certain new and useful Improvements in Compositions for Polishing Iron, of which the following is a specification.

My invention relates to a metal polish and 10 particularly to a composition of matter for removing rust and the like from iron.

Heretofore it has been a common practice to remove rust from iron by the use of abrasives and particularly by the use of sand 15 paper, or by dipping it into an acid such, for example, as sulfuric acid.

I have discovered that rust can be removed 20 from iron and the metal given a satisfactory polish by the application of a composition hereinafter set forth containing ingredients 25 which react chemically as described, with components of the rusted surface whereby such surface may be easily rendered clean and bright.

25 In the preparation of my polishing composition I employ a salt formed by uniting a weak base and a strong acid such, for example, as ammonium chlorid, ammonium sulfate, alum or the like. To this I add a 30 powdered metal which has a stronger ionizing tendency than that of iron such, for example, as zinc, magnesium, and aluminum. To this I preferably add an abrasive powder 35 of a high degree of hardness such as powdered rock crystal, powdered topaz, or the like.

The following is an example of the composition of my polishing powder in its preferred form:

|                                    | Parts by weight. |
|------------------------------------|------------------|
| Powdered metallic aluminum         | 2                |
| Dehydrated alum                    | 3                |
| Finely powdered crystalline silica | 5                |

45 In the use of my composition the powder is preferably applied to a water soaked cloth and rubbed steadily on the surface of the iron to be cleaned and polished. The rust gradually disappears and by continued action a 50 brilliantly polished surface results. The polished surface is then wiped off to remove the adhering composition and water and a suitable grease such as vaseline or the like may then be advantageously applied thereto 55 to preserve the polish. As my composition

is in the form of powder, its constituents are in contact and capable of reacting freely with each other and the iron rust upon the application of water.

The explanation of the polishing action 60 of my composition is believed to be as follows:

The salt is dissolved by the water on the cloth and in contact with the powdered metal disassociates, the negative ion of the 65 salt combining with the metal in the powder, and hydrogen in a nascent state being liberated in contact with the rust on the surface of the iron. This nascent hydrogen acting upon the iron oxid reduces it where- 70 by its easy removal is rendered possible.

It is advantageous to employ an abrasive powder such as powdered crystal silica to scratch the rust or oxidized surface of the metal whereby the action described is more 75 readily effected.

It is known that certain metals, such for example as zinc, can be deposited upon iron by the action of a third metal which is electro positive with respect to iron, in the 80 presence of a salt capable of producing an aqueous electrolyte when brought into contact with water. My invention is however distinguished from this metal coating process and composition employed therein as 85 I employ no coating metal nor, in fact, any metal capable of being deposited on the iron by the metal having a greater ionizing tendency on the salt employed than iron.

Having described my invention, I claim: 90

1. A composition of matter for cleaning and polishing iron, which comprises a salt of a strong acid and a weak base, an uncoated finely-divided metal having a greater ionizing tendency thereon than iron, and an 95 abrasive powder, said composition having the said ingredients thereof in intimate contact and capable of reacting freely with each other and with the iron rust and adapted upon the addition of moisture to remove rust 100 from iron with which it is placed in contact, said composition being free from any metal capable of being deposited on the iron by the action of the said finely divided metal.

2. A composition of matter for cleaning and polishing iron, which comprises three parts by weight of dehydrated alum, two parts by weight of finely-divided uncoated metallic aluminum, and five parts by weight 110

of powdered crystalline silica, said composition having the ingredients thereof in intimate contact and capable of reacting freely with each other and with the iron rust and 5 adapted upon the addition of moisture to remove rust from iron with which it is placed in contact, such composition being free from any metal capable of being de-

posited on the iron by the action of the said finely divided metal.

10

In testimony whereof I affix my signature in presence of two witnesses.

MATAICHI YASUDA.

Witnesses:

RYOKICHI OKUYAMA,  
HIDESABURO SEKI.